

March 15, 1927.

W. E. RUDER

1,621,380

PROCESS FOR MANUFACTURING SHEET METAL

Filed May 28, 1924



Fig. 2.



Fig. 3.



Fig. 4.



Inventor:  
William E. Ruder,

by *Alexander S. Lane*  
His Attorney.

Patented Mar. 15, 1927.

1,621,380

# UNITED STATES PATENT OFFICE.

WILLIAM E. RUDER, OF SCHENECTADY, NEW YORK, ASSIGNOR TO GENERAL ELECTRIC COMPANY, A CORPORATION OF NEW YORK.

## PROCESS FOR MANUFACTURING SHEET METAL.

Application filed May 28, 1924. Serial No. 716,522.

The present invention relates to the manufacture of sheet material and particularly to the production of sheet steel suitable for use in electric apparatus for the construction 5 of magnetic cores.

It has been the practice heretofore in the manufacture of sheet metal to cast the molten metal into the form of large ingots which are converted by a rolling mill into an 10 elongated bar of smaller cross-section. This bar is cut into lengths known as sheet bars which are of a size suitable for rolling into sheets. In the casting of the large ingots difficulties are experienced due to the formation 15 of a hollow center or "pipe". Apparently the solidification of the outer layer of metal while the interior is still molten leaves one or more central cavities by the contraction of the solidifying metal. The impurities 20 remaining in the molten metal also tend to segregate at the interior portion. Hence, it was necessary to discard an end portion of each ingot in which the piping was most pronounced. Usually a portion 25 of the remainder of the ingot which was rolled down to sheet form contained some cavities which caused a laminated structure in the sheet metal made therefrom.

Instead of casting large ingots requiring 30 an expensive rolling operation in order to produce bars suitable for rolling into sheets and entailing the removal of defective metal, I have provided in accordance with my present invention a new process whereby the 35 molten metal is cast into the form of a hollow cylinder in a mold rotatable at high speed so as to distribute the metal by centrifugal force. The resulting cast cylinder is subdivided into bars suitable for rolling into 40 sheets. This process therefore entirely eliminates the difficulties due to the formation of a cavity or cavities in the casting and eliminates the rolling operation formerly required to convert the large ingots into bars 45 from which sheets can be rolled.

My invention will be described in greater detail in the following specification taken in connection with the accompanying drawing, in which Fig. 1 is an elevation partly in section 50 of the casting apparatus, Fig. 2 is an end view partly in section of the casting mold, Fig. 3 is a perspective view of a casting produced in accordance with my invention

and Fig. 4 shows the casting subdivided or broken apart into bars suitable for subsequent rolling.

As shown in Fig. 1 the casting cylinder 1 in which castings are made is supported upon a horizontal shaft 2 which is rotatably mounted upon bearings 3 and 4, mounted on standards 5, 6. The mold is rotated by any suitable sorts of power belted to a pulley 7. The casting device comprises a cylindrical mold 8 preferably consisting of cast iron. This mold is connected by bolts or other suitable means to a frame 9, which is mounted upon the shaft 2. Surrounding the mold 8 is an enclosing shell 10 which is separated from the container 8 by a layer 11 of heat insulating material. Surrounding the rotatable mold is a protective shield 12. Removably bolted to the rim of the outer shell 10 of the mold is an annular rim plate 13 which serves as an end wall to hold the molten metal when it is distributed by centrifugal action against the interior wall of the rotating mold.

As shown in the drawing the molten metal is supplied to the mold by a ladle 14 which is mounted by a horizontal shaft 15 upon a wheeled truck 16. By means of this ladle the molten metal may be carried from the melting furnace to the mold. By tilting the ladle through rotation of the shaft 15, the molten charge is introduced into the 85 mold 1.

The mold 1 is rotated at a speed of about 400 to 500 revolutions per minute, the mold being brought up to speed before the molten charge is introduced. The molten metal is 90 spread out by centrifugal force as a layer of uniform thickness upon the interior surface of the mold. The centrifugal force causes impurities, such as slag or gases to 95 segregate upon the interior surface. The thickness of the casting may vary widely with conditions. I have obtained good results with mold castings 0.4" in thickness.

As best shown in Fig. 2 the interior surface of the cast iron 8 is provided with ridges or projections 18 spaced at regular intervals. These ridges which preferably are parallel with the longitudinal axis of the mold, produce corresponding indentations in 105 the surface of the cylindrical casting as in-

dicated at 19 in Fig. 3. These indentations, where the cross section of the metal is reduced, are convenient for subdividing the cast cylinder into longitudinal segments, particularly when the cast metal consists of silicon steel which is relatively brittle. In that case the indented cylindrical casting can be broken by properly applied blows into a number of segments as indicated in Fig. 4. Instead of breaking up the cylinder as described, it may be sub-divided by shearing or cutting, preferably while the casting is hot.

The segments 20 shown in Fig. 4 as being piled against each other are slightly curved, substantially rectangular plates which can be directly fed in the rolling mill and converted into sheets. In the rolling process

impurities on the surface of the bars 20 will be separated from the sheet as scale. 20

Although I have referred particularly to the production of silicon steel sheets, my process may be applied to the production of sheet metal of any character.

What I claim as new and desire to secure 25 by Letters Patent of the United States, is:

The method of manufacturing metal blanks preliminary to rolling into sheets which consists in casting molten metal into cylindrical form having a plurality of longitudinal grooves, and fracturing the metal in line with said grooves to separate said cylinder into a plurality of segments. 30

In witness whereof, I have hereunto set my hand.

WILLIAM E. RUDER.